# EUROPEAN PATENT APPLICATION

(11) **EP 4 786 618 A1**
(43) Date of publication of application: **05.08.2026**
(21) Application number: 24872165.6
(22) Date of filing: 24.09.2024
(51) Int. Cl.: C22C 38/00, C21D 6/00, C21D 8/00, C21D 8/06, C21D 9/00, C22C 38/58

(54) **PRECIPITATION-STRENGTHENED AUSTENITIC STAINLESS STEEL, PRODUCTION METHOD THEREFOR, AND COMPONENT FOR HYDROGEN ENVIRONMENT**

(30) Priority: 28.09.2023 JP 2023168602; 08.03.2024 JP 2024036250
(71) Applicant: Proterial, Ltd., Tokyo 135-0061 (JP)
(72) Inventor: GOTO, Ryosuke, Tokyo 135-0061 (JP); IBARA, Munehito, Tokyo 135-0061 (JP)
(74) Representative: HGF
(86) International application number: PCT/JP2024/033897
(87) International publication number: WO 2025/070374

(57) **Abstract**

A precipitation-strengthened austenitic stainless steel having less anisotropy in elongation and reduction in area in the material and having improved hydrogen-embrittlement resistance, and a manufacturing method for the precipitation-strengthened austenitic stainless steel are provided. A precipitation-strengthened austenitic stainless steel consisting of, in mass %, up to 0.08% C, up to 1.00% Si, up to 2.00% Mn, up to 0.040% P, up to 0.030% S, 24.00-27.00% Ni, 13.50-16.00% Cr, 1.00-1.50% Mo, 1.90-2.35% Ti, up to 0.35% Al, 0.10-0.50% V, 0.001-0.010% B, and the balance being Fe and inevitable impurities, wherein the Ti segregation ratio in the material is 1.25 or less, a manufacturing method for the precipitation-strengthened austenitic stainless steel, and a component for a hydrogen environment are provided.

## Description

### TECHNICAL FIELD

The present invention relates to precipitation-strengthened austenitic stainless steel and to manufacturing methods therefor, and to components for hydrogen environments.

### BACKGROUND ART

Efforts toward achieving a decarbonized society have been globally made against a background of recent environmental issues. Among these efforts, practical use of fuel cell vehicles that do not emit carbon dioxide and that use hydrogen gas, and practical use of hydrogen stations as infrastructure for the fuel cell vehicles have attracted attention.

In order to put fuel cell vehicles and hydrogen stations into practical use, hydrogen gas containers, pipes, instruments, etc., are necessary, and therefore, metal materials having high strength and hydrogen-embrittlement resistance suitable for these applications are necessary. These metal materials are defined under High Pressure Gas Safety Act, and SUS316, SUS316L, SCM435, SUH660, XM-19, etc., have been selected based on exemplary standards for the General High-Pressure Gas Safety Regulations. These are materials of which performance has been evaluated by calculating the relative ratio between mechanical properties in air and mechanical properties in a hydrogen environment and of which hydrogen-embrittlement resistance has been recognized as being excellent from the evaluation results.

Among these metal materials, SUH660 having the highest strength is used for components which are used in hydrogen environments and for which strength is particularly required. SUH660 is a precipitation-strengthened austenitic steel defined by Japanese Industrial Standards (hereinafter, JIS). By performing a solution and aging treatment, the gamma prime phase can be coherently precipitated in the matrix of this material, and as a result, high strength can be achieved. Originally, this material has been developed as a heatresistant alloy steel, and it is known to have excellent hydrogen-embrittlement resistance in a temperature range from -253°C or more and 120°C or less and under a hydrogen gas pressure of 82 MPa or less. In addition, in the Patent Documents in Reference Document List, there have been proposed inventions to further improve mechanical properties, etc., of an SUH660-equivalent steel and an alloy steel having a composition similar thereto.

For example, the applicant of the present application has proposed, in Patent Document 1, a manufacturing method including performing hot forging on a forging material of a precipitation-strengthened austenitic alloy such that the total forging ratio is 30 or greater. According to this invention, mechanical properties can be improved, and an increased service life of components can be expected under a high-pressure hydrogen environment.

Patent Document 2 states that both high strength and hydrogen-embrittlement resistance can be achieved by introducing dislocations into Fe-Ni-based alloys through cold working so as to increase the tensile strength to 1000 MPa or more while limiting the upper limit of the tensile strength to 1300 MPa.

Patent Document 3 states that high strength can be achieved by enabling austenitic stainless steel to contain Ti, by setting No. 8 or greater as the grain size, and by controlling the η phase precipitated at the grain boundary. Patent Document 3 states that a tensile strength of 1150 MPa or greater can be stably obtained without causing hydrogen embrittlement.

Patent Document 4 states that hot workability, tensile strength, and hydrogen-embrittlement resistance can be achieved by adding rare-earth elements to stainless steel.

### REFERENCE DOCUMENT LIST

### PATENT DOCUMENTS

| | |
|---|---|
| Patent Document 1: | WO 2023/145423 |
| Patent Document 2: | JP 2011-68919 A |
| Patent Document 3: | JP 2014-47409 A |
| Patent Document 4: | JP 2018-95929 A |

### SUMMARY OF THE INVENTION

### PROBLEM TO BE SOLVED BY THE INVENTION

Each of the above-described Patent Documents is directed to a SUH660-equivalent steel or a precipitation-strengthened austenitic stainless steel similar thereto, and one effect of the invention is to improve mechanical properties of such steel. In addition, in these inventions, a tensile test specimen is sampled from a certain location of a target material, a tensile test is conducted on the tensile test specimen, and mechanical properties of the tensile test specimen are evaluated. In addition, the evaluation results are presented as representative values of the material. Thus, it is desirable that the representative values of the mechanical properties should not depend largely on the sampling location or the sampling direction of the test specimen sampled from the material. In addition, when mechanical properties of an alloy are evaluated by a tensile test, in many cases, a tensile test specimen is normally sampled in the longitudinal direction of the material, taking the length of the test specimen into account. That is, this direction matches the forging direction in the hot forging step when the material is manufactured, and it is often the case that the mechanical properties in the forging direction are adopted as the representative values of the material.

In order to evaluate the anisotropies in the mechanical properties in a material, the present inventors sampled two tensile test specimens from a single material, one in the compression direction and the other in the forging direction of the material. Mechanical properties of these two tensile test specimens at room temperature in air were compared with each other, and were evaluated. As a result, the present inventors found that even when a material, which exhibits no anisotropy in 0.2% yield strength and tensile strength, exhibits anisotropy in elongation and reduction in area.

When anisotropy is observed in elongation and reduction in area at room temperature and atmospheric pressure, it is necessary to set, for example, a large safety factor to the representative values of the mechanical properties, and product design using this material may be significantly hindered. In addition, as described above, the performance of the hydrogen-embrittlement resistance is evaluated by calculating the relative ratio between the mechanical properties in air and the mechanical properties in a hydrogen environment. Thus, when anisotropy is observed in elongation and reduction in area of a material, it means that there is also anisotropy in hydrogen-embrittlement resistance. This anisotropy may cause a significant problem when the material is used in a hydrogen environment. This problem regarding the anisotropy in elongation and reduction in area has not been recognized in the Patent Documents, leaving room for further investigation. Thus, it is an object of the present invention to provide a precipitation-strengthened austenitic stainless steel having less anisotropy in elongation and reduction in area in the material and having improved hydrogen-embrittlement resistance.

### MEANS FOR SOLVING THE PROBLEM

In order to solve the problem with the anisotropy in elongation and reduction in area of an SUH660 material, the present inventors observed and analyzed the microstructure of this material in detail, and investigated the causes of the anisotropy. As a result, the present inventors found that banded segregation was present in the microstructure obtained after a hot-forged steel billet (billet) was subjected to solution and aging treatment. As a result of extensive studies, the present inventors found that the anisotropy in elongation and reduction in area can be significantly improved by reducing this banded segregation, found a manufacturing method effective to reduce the banded segregation, and arrived at the present invention.

That is, in one aspect of the present invention, there is provided a precipitation-strengthened austenitic stainless steel consisting of, in mass %, up to 0.08% C, up to 1.00% Si, up to 2.00% Mn, up to 0.040% P, up to 0.030% S, 24.00-27.00% Ni, 13.50-16.00% Cr, 1.00-1.50% Mo, 1.90-2.35% Ti, up to 0.35% Al, 0.10-0.50% V, 0.001-0.010% B, and the balance being Fe and inevitable impurities, wherein the Ti segregation ratio in the steel is 1.25 or less.

In addition, in another aspect of the present invention, there is provided a manufacturing method for the above-described precipitation-strengthened austenitic stainless steel, the manufacturing method including: a first homogenization heat treatment step of performing a homogenization heat treatment on a prepared steel ingot at a heating temperature of 980 to 1270°C, to obtain a hot-forging material; a hot forging step of performing hot forging on the hot-forging material, to obtain a steel billet; and a solution and aging treatment step of performing a solution treatment and an aging treatment on the steel billet, wherein the heat treatment time of the first homogenization heat treatment is 25 to 150 hours.

Preferably, the manufacturing method includes a second homogenization heat treatment step of performing a homogenization heat treatment on at least one of the steel billet and an intermediate material obtained during the hot forging at a heating temperature of 980 to 1270°C, wherein the total heat treatment time of the first homogenization heat treatment and the second homogenization heat treatment is 25 to 150 hours.

In addition, in another aspect of the present invention, there is provided a component for a hydrogen environment, the component being made of the above-described precipitation-strengthened austenitic stainless steel.

### EFFECTS OF THE INVENTION

According to the present invention, it is possible to provide a precipitation-strengthened austenitic stainless steel having less anisotropy in elongation and reduction in area in the material and having improved hydrogen-embrittlement resistance.

### BRIEF DESCRIPTION OF THE DRAWINGS

[FIG. 1] This figure schematically illustrates the sampling locations and the sampling directions of tensile test specimens sampled from a steel billet.
[FIG. 2] This figure illustrates the relationship between the total homogenization heat treatment time and the Ti segregation ratio.
[FIG. 3] This figure illustrates the relationship between the Ti segregation ratio and the elongation anisotropy ratio.
[FIG. 4] This figure illustrates the relationship between the Ti segregation ratio and the reduction-in-area anisotropy ratio.

### MODE FOR CARRYING OUT THE INVENTION

Hereinafter, an embodiment of the present invention will be described in detail. First, a precipitation-strengthened austenitic steel according to the present invention will be described. The precipitation-strengthened austenitic steel according to the present invention is an SUH660-equivalent alloy defined by JIS (Japanese Industrial Standards) G-4311, having a composition consisting of, in mass %, up to 0.08% C, up to 1.00% Si, up to 2.00% Mn, up to 0.040% P, up to 0.030% S, 24.00-27.00% Ni, 13.50-16.00% Cr, 1.00-1.50% Mo, 1.90-2.35% Ti, up to 0.35% Al, 0.10-0.50% V, 0.001-0.010% B, and the balance being Fe and inevitable impurities. Hereinafter, unless otherwise specified, the precipitation-strengthened austenitic stainless steel according to the present embodiment refers to the above-described SUH660-equivalent alloy.

A key feature of the precipitation-strengthened austenitic steel according to the present invention is that the Ti segregation ratio in the material is 1.25 or less. The significance of defining the Ti segregation ratio will be described. According to the analysis by the present inventors, banded segregation may be present in the microstructure after a steel billet (which is a semi-finished product obtained by cogging a steel ingot, and which may be referred to as a billet) of a precipitation-strengthened austenitic steel is subjected to a solution and aging treatment. It is generally known that banded segregation is formed when the solidification structure (dendritic structure) in a steel ingot (ingot) is compressed by hot forging. Because the dendritic structure has microsegregation, microsegregation is elongated in the forging direction during hot working, and banded segregation layers are consequently formed.

If banded segregation is formed on the precipitation-strengthened austenitic steel, Ni, Ti, Al, and other elements forming the gamma prime phase are unevenly distributed, and it is not possible to isotropically distribute the gamma prime phase after the aging treatment. Thus, it is considered that anisotropy in mechanical properties occurs between the compression direction and the forging direction. In particular, a continuous variation in the concentration of the gamma prime distribution occurs due to the banded segregation layers in the compression direction, which may deteriorate the mechanical properties. Among the mechanical properties, the anisotropy in 0.2% yield strength and tensile strength is more strongly affected by the grain size than by the distribution state of the gamma prime phase at room temperature. Thus, when the grains are isotropic, the influence of the banded segregation tends to be negligible. On the other hand, since the elongation and the reduction in area are strongly affected by the distribution state of the gamma prime phase, it is considered that anisotropy becomes more pronounced. Thus, by reducing the above-described banded segregation, it is expected that the anisotropy in elongation and reduction in area of precipitation-strengthened austenitic steel can be reduced.

Because the above-described banded segregation is formed when the dendritic structure is forged and compressively deformed, the thickness of each of the banded layers is less than that of the dendritic structure. For example, a secondary dendrite arm spacing, which is a representative size of the dendritic structure, is from several tens of micrometers to several hundreds of micrometers, and it is considered that the banded segregation formed by compressing the dendritic structure forms variations in concentration at intervals of several micrometers at minimum. Thus, in the present invention, by using an EPMA (electron probe microanalyzer), the local concentration distribution in the material is evaluated. In addition, as the element to be analyzed, Ti is selected, which is an element forming the gamma prime phase, and is a major constituent element of the precipitation-strengthened austenitic steel. Ti is selected because the equilibrium distribution coefficient is less and is easy to segregate. After the local concentration of Ti is analyzed at multi points with an EPMA, the Ti segregation ratio is obtained from the ratio of the maximum concentration with respect to the minimum concentration (maximum concentration/minimum concentration). In the present invention, the extent of the banded segregation in the material can be quantitively evaluated from this Ti segregation ratio.

In the present embodiment, when the local element concentration is measured with an EPMA, the probe diameter of the EPMA is determined in accordance with the distance between high and low concentration regions in the banded segregation. It is preferable that the probe diameter be in a range of 0.5 to 1.0 µm so as to avoid variations in composition caused by products other than solidification segregation, such as the gamma prime phase. In addition, to increase the accuracy of the analysis result, it is preferable that 100 or more data points be acquired from a single measurement target material. After removing the data outliers from the analysis result, the maximum Ti concentration and the minimum Ti concentration are obtained, and the ratio therebetween is derived as the segregation ratio. The data outliers are data points representing abnormally high Ti concentration. These data outliers are obtained when the analysis probe of the EPMA is positioned on a Ti carbide (TiC) or Ti nitride (TiN) present inside a grain or at a grain boundary, not the matrix in the microstructure of the material.

A key feature of the precipitation-strengthened austenitic stainless steel according to the present invention is that the above-described Ti segregation ratio is 1.25 or less. When the Ti segregation ratio is 1.25 or less, the banded segregation in the material is sufficiently rendered harmless, and accordingly, the anisotropy in elongation and the anisotropy in reduction in area, which are ductility indices, can be sufficiently reduced. The manufacturing process of the precipitation-strengthened austenitic stainless steel according to the present embodiment includes hot forging, and the anisotropy in mechanical properties is evaluated by the ratio of forging-direction characteristics with respect to compressiondirection characteristics. That is, the anisotropy in elongation is evaluated by the elongation anisotropy ratio obtained by "the elongation in the forging direction"/"the elongation in the compression direction", and the anisotropy in reduction in area is evaluated by the reduction-in-area anisotropy ratio obtained by "the reduction-in-area in the forging direction/the reduction-in-area in the compression direction". In the case of the precipitation-strengthened austenitic stainless steel according to the present embodiment, because the elongation anisotropy ratio and the reduction-in-area anisotropy ratio are each 1.60 or less, it is assumed that the anisotropy has been sufficiently reduced. The upper limit of the elongation anisotropy ratio is preferably 1.50, more preferably, 1.45. In addition, the upper limit of the reduction-in-area anisotropy ratio is preferably 1.58.

Next, a manufacturing method of the precipitation-strengthened austenitic stainless steel according to the present invention will be described.

First, a steel ingot (ingot) serving as a hot-forging material is prepared by melting. It is preferable that vacuum melting be used for this ingot according to the present embodiment. In order to prevent formation of macrosegregation, which is hard to render harmless in a subsequent process, it is preferable that remelting based on an electroslag remelting method or a vacuum arc remelting method be performed, using the melted ingot as a consumable electrode for remelting.

In the present embodiment, a first homogenization heat treatment is performed on the prepared ingot. This is to reduce microsegregation, which is the cause of banded segregation, as much as possible, and to homogenize the composition concentration distribution in the material. By performing the homogenization heat treatment at the ingot stage, it is possible to obtain an effect of preventing cracking from occurring in the subsequent hot forging process. The temperature of the homogenization heat treatment is set to a solidus temperature or less and a solution treatment temperature or more. The reason the temperature is set to the solidus temperature or less is that a temperature above the solidus temperature may result in local melting in the material. The reason the temperature is set to the solution treatment temperature or more is to completely dissolve the precipitates formed during cooling after solidification into the matrix. In order to sufficiently obtain the effect of the present invention, it is necessary to set the Ti segregation ratio to 1.25 or less, and a suitable temperature of the homogenization heat treatment for this purpose is 980°C to 1270°C, and more preferably, 1100°C to 1200°C. It is important that the heat treatment time be set as a total heat treatment time (which will be also referred to as "total homogenization heat treatment time"), which is obtained by adding a second homogenization heat treatment time performed at a billet stage described below, in order to obtain the effect of the present invention. It is preferable that the total homogenization heat treatment time be 25 hours or more, and more preferably, 30 hours or more. As the total homogenization heat treatment time extends, the banded segregation reduction effect saturates. In addition, because execution of the heat treatment for a long time deteriorates manufacturability, it is preferable that the total homogenization heat treatment time be set to 150 hours or less, and more preferably, 100 hours or less. The total homogenization heat treatment time is represented by the following equation. Total homogenization heat treatment time = Ingot-stage homogenization heat treatment time + Billet-stage homogenization heat treatment time

If the Ti segregation ratio can be set to 1.25 or less by the ingot-stage homogenization heat treatment alone, because the formation of the banded segregation becomes negligible, the effect of the present invention can be obtained sufficiently, even if the microstructure is compressed by the subsequent hot forging. Thus, in this case, the homogenization heat treatment does not need to be performed at the billet state.

In the present embodiment, hot forging is performed on the hot-forging material obtained after the first homogenization heat treatment, to manufacture a billet having predetermined cross-sectional dimensions. It is preferable that a second homogenization heat treatment be performed as needed. Specifically, a homogenization heat treatment is performed on an intermediate material obtained during the hot forging process or a billet obtained after the hot forging. When the second homogenization heat treatment is performed, the diffusion distance of the segregated solute element can be shortened by compressing and deforming the dendritic solidification structure of the ingot. Thus, a high homogenization effect can be obtained when the dendritic structure is coarse, such as at the central axis portion of a large-size ingot. The billet-stage homogenization heat treatment temperature is preferably 980°C to 1270°C, and more preferably, 1100°C to 1200°C. The second homogenization heat treatment time may be set as appropriate based on the above-described total homogenization heat treatment time. Whether to perform the second homogenization heat treatment during or after the hot forging process may be determined in view of the grain size required for the final material product. When a material compression process such as die forging or cold forging is not included after the hot forging process, the grain size needs to be large by the end of the hot forging for addition of strength. Thus, it is preferable that the second homogenization heat treatment be performed during the hot forging. Even when the second homogenization heat treatment is performed, if the first homogenization heat treatment is not performed on the ingot, a crack may occur during the hot forging due to segregation. Thus, it is necessary to perform the first homogenization heat treatment in the manufacturing method according to the present invention.

In the present embodiment, in order to sufficiently increase the strength of the material, a solution and aging treatment is performed on a billet. The reason the solution treatment is executed is to dissolve the precipitates, which have been generated during the cooling after the solidification or during the cooling after the hot forging, in the matrix. The reason the aging treatment is executed is to coherently precipitate the gamma prime phase in the matrix and to sufficiently improve the strength of the material. The heat treatment temperature of the solution treatment is preferably 850°C to 1050°C, more preferably, 900°C to 1000°C. The heat treatment temperature in the aging treatment is preferably 650°C to 800°C, more preferably, 700°C to 760°C.

Components for hydrogen environments, the components being made of the precipitation-strengthened austenitic stainless steel according to the present invention, are expected to exhibit good mechanical properties. These "components for hydrogen environments" can be applied to components for fuel cell vehicles and hydrogen stations, the components being exposed to high-pressure hydrogen gas. Examples of such components include piping, tanks, valves, and dispenser components.

### Examples

### (Example 1)

Four ingots (materials Nos. 1 to 4), each of which weighs approximately 10 kg and has a chemical composition shown in Table 1, were melted in a vacuum melting furnace. The chemical compositions fall within the range of chemical compositions of SUH660 defined by JIS. Next, in order to reduce microsegregation, the first homogenization heat treatment was performed on these ingots, and a different heat treatment time between 1140°C and 1200°C was set for each ingot. As the heat treatment time, 5 hours was set for material No. 1; 35 hours for material No. 2; 45 hours for material No. 3; and 20 hours for the material No. 4.

**[Table 1]**

| (mass %) | | | | | | | | | | | | | |
|---|---|---|---|---|---|---|---|---|---|---|---|---|---|
| Material No. | C | Si | Mn | P | S | Ni | Cr | Mo | Ti | Al | B | v | Balance |
| 1 | 0.04 | 0.03 | 50.01 | 0.004 | 0.002 | 25.6 | 14.72 | 1.36 | 2.21 | 0.30 | 0.003 | 0.29 | Fe and Inevitable impurities |
| 2 | 0.04 | 0.01 | 50.01 | 0.004 | 0.002 | 24.5 | 14.28 | 1.29 | 2.12 | 0.29 | 0.004 | 0.27 | Fe and Inevitable impurities |
| 3 | 0.04 | 0.03 | 50.01 | 0.004 | 0.002 | 25.5 | 14.91 | 1.35 | 2.20 | 0.30 | 0.004 | 0.29 | Fe and Inevitable impurities |
| 4 | 0.04 | 0.02 | 50.01 | 0.003 | 0.002 | 25.6 | 14.76 | 1.42 | 2.26 | 0.33 | 0.003 | 0.33 | Fe and Inevitable impurities |

After the first homogenization heat treatment, hot forging was performed on the ingot materials of material Nos. 1 to 4 at 1000°C or more, and four bar-shaped billets having a diameter of approximately 30 mm and a length of 1000 mm were manufactured. Among the manufactured billets, only the bar-shaped billet manufactured from the ingot of material No. 4 was divided transversely, to obtain a total of seven billet materials. In addition, in order to reduce banded segregation, a homogenization heat treatment was performed on six of these seven billets at a temperature between 1100°C to 1200°C for 10 hours to 60 hours. As a result, the total homogenization heat treatment time for the materials on which the homogenization heat treatment was executed at the billet stage ranged from 30 hours to 80 hours.

Next, for all the billets obtained from the ingot materials of material Nos. 1 to 4, a solution treatment and an aging treatment were performed, to dissolve unnecessary precipitated phases and to precipitate the gamma prime phase. The heat treatment temperature of the solution treatment was set to 980°C, the heat treatment time was set to one hour, and the cooling was performed by oil cooling. In addition, the heat treatment temperature of the aging treatment was set to set to 718°C, the heat treatment time was set to 16 hours, and the cooling was performed by air cooling.

Tensile test specimens were sampled from the billets, on which the solution and aging treatment was performed, in two directions of the compression direction and the forging direction, as illustrated in FIG. 1. A tensile test specimen in the compression direction was sampled from a location such that the center point of the test specimen and the center point of a cross section of the billet match. A tensile test specimen in the forging direction was sampled from a location such that a location corresponding to D/4 (D denotes the diameter) of a cross section of the billet and the center point of a cross section of the test specimen match. The tensile test specimen in the compression direction and the tensile test specimen in the forging direction had the same dimensions, and each of these tensile test specimens was processed into a round-bar tensile test specimen having a gauge diameter of 2.5 mm and a gauge length of 10 mm. The tensile tests were performed at room temperature in air, and test conditions compliant with ASTM E8/E8M were selected. Under these conditions, tensile tests were performed on one billet element in the two directions of the compression direction and the forging direction. From the results of the tensile tests, the elongation anisotropy ratio and the reduction-in-area anisotropy ratio were derived. In the present Example, the acceptable levels of the elongation anisotropy ratio and the reduction-in-area anisotropy ratio were set to 1.50 or less.

Next, to obtain the Ti segregation ratio in the material, samples for EPMA analysis were collected from the billet materials on which the solution and aging treatment was performed, the analysis surface was mirror-polished, and quantitative analysis of the Ti concentration was performed with an EPMA. The EPMA analysis was performed under the following conditions: an accelerating voltage of 15 kV, an incident beam current of 100 nA, an analysis time of 1 s per point, a probe diameter of 1 µm, 100 analysis points arranged in a square grid, and an analysis area of 1 mm × 1 mm. The segregation ratio was obtained as the ratio of the maximum Ti concentration with respect to the minimum Ti concentration. However, when analysis points coincided with Ti carbides or Ti nitrides that crystalized during solidification and remained in their billet, extremely high Ti concentrations were obtained. Thus, data that showed a Ti concentration more than the Ti content of the corresponding material in Table 1 by 0.24% or higher was considered as an outlier, and was excluded from the dataset used to determine the segregation ratio. The results are shown in Table 2.

**[Table 2]**

| Sample No. | Material No. | First heat treatment time (hr) | Second heat treatment time (hr) | Total heat treatment time (hr) | Ti segregation ratio | Elongation anisotropy ratio | Reduction-in-area anisotropy ratio | Evaluation of anisotropy | Category |
|---|---|---|---|---|---|---|---|---|---|
| 1 | 1 | 5 | 0 | 5* | 1.41* | 1.71 | 1.66 | X | Comparative example |
| 2 | 4 | 20 | 0 | 20* | 1.30* | 1.99 | 1.74 | X | Comparative example |
| 3 | 4 | 20 | 10 | 30 | 1.22 | 1.09 | 1.22 | ✔ | Inventive example |
| 4 | 2 | 35 | 0 | 35 | 1.16 | 0.91 | 0.92 | ✔ | Inventive example |
| 5 | 4 | 20 | 20 | 40 | 1.14 | 1.42 | 1.19 | ✔ | Inventive example |
| 6 | 3 | 45 | 0 | 45 | 1.20 | 1.15 | 1.56 | ✔ | Inventive example |
| 7 | 4 | 20 | 30 | 50 | 1.10 | 0.74 | 0.95 | ✔ | Inventive example |
| 8 | 4 | 20 | 40 | 60 | 1.09 | 1.04 | 1.13 | ✔ | Inventive example |
| 9 | 4 | 20 | 50 | 70 | 1.08 | 1.30 | 1.00 | ✔ | Inventive example |
| 10 | 4 | 20 | 60 | 80 | 1.13 | 0.99 | 1.08 | ✔ | Inventive example |

| | | | | | | | | | |
|---|---|---|---|---|---|---|---|---|---|
| "*" indicates that the data is outside the range defined by the present invention. | | | | | | | | | |

Sample No. 1 and sample No. 2 are comparative examples in which the homogenization heat treatment was performed at the ingot stage for five hours or 20 hours, and the total heat treatment time was less than 25 hours. As shown in Table 2, it was found that the homogenization was insufficient, the Ti segregation ratio exceeded 1.25, and the elongation anisotropy ratio and the reduction-in-area anisotropy ratio did not reach their target. For sample No. 4 and sample No. 6, the homogenization heat treatment was also performed at their ingot stage, but the total homogenization heat treatment time was set to 25 hours or more for either sample. It was found that a sufficient homogenization was reached, and the Ti segregation ratio was below 1.25 for each of the samples. Thus, the elongation anisotropy ratio and the reduction-in-area anisotropy ratio were both low values below their target value 1.60, which is the allowable level of anisotropy. Thus, the effect of the present invention was sufficiently obtained.

In addition, for samples No. 3, No. 5, and No. 7 to No. 10, the homogenization heat treatment was performed at the ingot stage and at the billet stage, in either of which, the total homogenization heat treatment time was set to 25 hours or more. It was found that a sufficient homogenization was achieved, and the Ti segregation ratio was below 1.25 for each of the samples. Thus, the elongation anisotropy ratio and the reduction-in-area anisotropy ratio were both low values below their target value 1.60, which is the allowable level of anisotropy. Thus, it was confirmed that the effect of the present invention can be sufficiently obtained.

FIG. 2 illustrates the relationship between the total homogenization heat treatment time and the Ti segregation ratio. It was confirmed from FIG. 2 that the Ti segregation ratio tends to decrease as the total homogenization heat treatment time is longer. In addition, by approximating the relationship between the total homogenization heat treatment time and the Ti segregation ratio by a quadratic polynomial, it was confirmed that at least 25 hours is needed as the total homogenization heat treatment time to bring the Ti segregation ratio to be 1.25 or less.

FIG. 3 shows the relationship between the Ti segregation ratio and the elongation anisotropy ratio, and FIG. 4 shows the relationship between the Ti segregation ratio and the reduction-in-area anisotropy ratio. It is seen from FIG. 3 that the correlation coefficient between the Ti segregation ratio and the elongation anisotropy ratio is 0.72, which indicates a positive correlation, and that the elongation anisotropy ratio tends to decrease as the Ti segregation ratio decreases. It is also seen from FIG. 4 that the correlation coefficient between the Ti segregation ratio and the reduction-in-area anisotropy ratio is 0.85, which indicates a positive correlation, and that the reduction-in-area anisotropy ratio tends to decrease as the Ti segregation ratio decreases. Thus, it was confirmed that the inventive precipitation-strengthened austenitic stainless steel of which the Ti segregation ratio is 1.25 or less exhibits a low elongation anisotropy ratio and a low reduction-in-area anisotropy ratio and has excellent mechanical properties without anisotropy.

## Claims

1. A precipitation-strengthened austenitic stainless steel consisting of, in mass %, up to 0.08% C, up to 1.00% Si, up to 2.00% Mn, up to 0.040% P, up to 0.030% S, 24.00-27.00% Ni, 13.50-16.00% Cr, 1.00-1.50% Mo, 1.90-2.35% Ti, up to 0.35% Al, 0.10-0.50% V, 0.001-0.010% B, and the balance being Fe and inevitable impurities, wherein a Ti segregation ratio in the steel is 1.25 or less.

2. A manufacturing method for the precipitation-strengthened austenitic stainless steel according to claim 1, the manufacturing method comprising:
a first homogenization heat treatment step of performing a homogenization heat treatment on a prepared steel ingot at a heating temperature of 980 to 1270°C, to obtain a hot-forging material;
a hot forging step of performing hot forging on the hot-forging material, to obtain a steel billet; and
a solution and aging treatment step of performing a solution treatment and an aging treatment on the steel billet,
wherein heat treatment time of the first homogenization heat treatment is 25 to 150 hours.

3. The manufacturing method for the precipitation-strengthened austenitic stainless steel according to claim 2, the manufacturing method comprising a second homogenization heat treatment step of performing a homogenization heat treatment on at least one of the steel billet and an intermediate material obtained during the hot forging at a heating temperature of 980 to 1270°C, wherein a total heat treatment time of the first homogenization heat treatment and the second homogenization heat treatment is 25 to 150 hours.

4. A component for a hydrogen environment, the component being made of the precipitation-strengthened austenitic stainless steel according to claim 1.
